# EUROPEAN PATENT SPECIFICATION

(11) **EP 0 259 940 B1**
(45) Date of publication and mention of the grant of the patent: **22.07.1992**
(21) Application number: 87201796.7
(22) Date of filing: 14.09.1987
(51) Int. Cl.: E01C 13/00, A63C 19/04

(54) **Method of manufacturing an artificial grass and an artificial grass obtained therewith**
Verfahren zur Herstellung von Kunstgras und dadurch hergestelltes Kunstgras
Procédé de fabrication d'une herbe artificielle, et herbe artificielle ainsi obtenue

(30) Priority: 12.09.1986 NL 8602312
(43) Date of publication of application: 16.03.1988
(73) Proprietor: Koninklijke Nijverdal-Ten Cate N.V., NL-7607 GB Almelo (NL)
(72) Inventor: Terhorst, Antonius Vincentius, NL-7576 EM Oldenzaal (NL); van den Bosch, Harm, NL-7607 HA Almelo (NL)
(74) Representative: Schumann, Bernard Herman Johan

(56) References cited:
- EP-A- 0 099 047
- EP-A- 0 244 486
- DE-A- 1 504 110
- DE-A- 2 015 355
- DE-A- 2 512 707
- FR-A- 2 187 530
- FR-A- 2 238 805
- US-A- 3 940 522
- US-A- 4 061 804
- US-A- 4 337 283
- US-A- 4 348 434

## Description

The invention relates to a method for manufacturing artificial grass, consisting of an underlayer and strip-like pile threads embedded therein, which threads protrude, as grass, on one side out of the underlayer and wherein as raw material for the threads use is made of a polymer. The invention also relates to artificial grass obtained by the above method.

Such a method is known from e.g. US-A-4 337 283.

It is a purpose of the invention to provide a method of the type mentioned in the preamble, by means of which artificial grass may be manufactured having a structure including a smoothing agent forming part of the threads. Such construction results in a grass surface that does not necessarily require an after-treatment or a regular or periodic servicing.

To this end the method according to the invention is characterized in that to said raw material a second material having a different composition and reducing the coefficient of friction is added.

In a specific embodiment the method is characterized in that the raw material is a polypropylene.

The Nederlandse Sportfederatie (NSF) (Dutch Sport Federation) among others lays down particular requirements with respect to the characteristics of artificial grasses, including requirements related to the coefficient of friction. The NSF together with the Koninklijke Nederlandse Voetbalbond (Football Association) has adopted the standards 2.a, 4.b, 4.c and 4.d applicable to soccer. In such a "Leroux" test the coefficient of friction is expressed in terms of roughness. This roughness can be expressed in one characterizing number and must be as low as possible. In principle a value of at the highest 0.3 is required for a soccer pitch.

Additionally, use can be made of frizzing or crinkles to obtain the isotropic properties of the turf. An effective lowering of the coefficient of friction can be realized in this way. Use can be made for this purpose of a circle knit method or knit-deknit. The crinkles can be fixed in a furnace, for example by means of hot air or steam. Use can be made for instance of at least one treatment at a temperature of approximately 130°C for a time period in the order of 10 minutes. It can be useful, depending on the materials employed, to repeat such a thermal treatment several times.

Polyethylene terephthalate or polytetrafluoroethylene can for example be added in a ratio in the order of 50% : 50%. Other substances can also be used. Special mechanical techniques can also be employed in the manufacture of the threads, for instance a coextrusion of a number, e.g. 3 or 5, of films onto one another, including for example at least one moisture absorbing layer. Even "super absorbers" can be applied in this context. The function of a moisture absorbing layer is to take up moisture and release it at the moment when the pitch has to be played on, which results in a lowered coefficient of friction being brought about owing to the released moisture, also in dry weather.

A laminate type structure, for example 3 co-extruded films, can consist of a centre layer of the relatively rigid polypropylene with a thickness of 60%, having on either side a layer with a thickness of 20% and consisting of another more flexible material, for example linear low density polyethylene. Also use can be made of polyethylene terephthalate. This material possesses a low coefficient of friction and also has a (small) moisture absorption capacity.

An after-treatment can be applied for addition of smoothing substances as coating layer on the pile threads, for example consisting of polytetrafluoroethylene and/or material on a silicon base. Strips can be treated in the factory. A watery dispersion of smoothing substance can be manufactured and applied to the threads by spraying or another suitable process, and the water allowed to evaporate. The strip-like threads can thus for example be guided beforehand through a dispersion of the smoothing material, or a field with artificial grass can be rolled with a roller running through a liquid bath.

### Example 1

Use was made of threads consisting of approximately 90% polypropylene, approximately 8% linear low density polyethylene and approximately 2% CaCO₃, in addition to small quantities of the additions that are further usual to improve the mechanical, thermal and ultra violet stability and the like. Addition of CaCO₃ gives an increase in stiffness and lessens the tendency of the pile threads to splitting.

Use was made of a three-strand thread 3 x 2200 DTEX twine, 5 mm x 50 µ.

Thread frizzed.

### Example 2

Threads as in example 1, frizzed. Frizzing length 20-30 mm. Frizzing fixed with steam, 130°C for 2 x 10 minutes.

### Example 3

Thread as specified above, fibrillated with four needles per centimetre, incision length 8 - 12 mm.

### Example 4

Application of coating layer. Thread as specified above. For smoothing the threads use is made of a surface treatment agent. Surface treatment means the applying of a liquid to give the thread the desired properties with respect to its processing and final characteristics. A surface treatment agent can if necessary permeate into the thread through diffusion. In this case the surface treatment agent consisted of a mixture of silicon oils and polytetrafluoroehtylene. The surface treatment agent was dispersed in water. The dispersion was sprayed on. After evaporation of the water there remained 1-2% active substance or surface treatment agent per kg. of pile thread.

### Example 5

A typical carpet construction for artificial football turf is manufactured on a tufting machine with 3/8 or 5/16 division, a stitch count of 14-16 per 10 cm and a pile height of 32-35 mm.

The standards referred to were satisfied in all cases.

## Claims

1. Method for manufacturing artificial grass, consisting of an underlayer and strip-like pile threads embedded therein, which threads protrude, as grass, on one side out of the underlayer and wherein as raw material for the threads use is made of a polymer, characterized in that to said raw material a second material having a different composition and reducing the coefficient of friction is added.

2. Method as claimed in claim 1, characterized in that the raw material is a polypropylene.

3. Method as claimed in claim 1, characterized in that polytetrafluoroethylene or polyethylene terephthalate is mixed with the polymer, for instance in the form of a masterbatch.

4. Method as claimed in claim 3, characterized in that the mixing ratio is selected in the order of magnitude of 50% : 50%.

5. Method as claimed in claim 3, characterized in that the quantity of polytetrafluoroethylene is chosen such that the resulting quantity thereof amounts to approximately 2-7% of the total thread weight.

6. Method as claimed in claim 1, characterized in that for manufacture of the threads both materials are extruded simultaneously.

7. Method as claimed in any of the foregoing claims, characterized in that threads are manufactured by coextrusion of a number of films in order to obtain the required mechanical properties, such as coefficient of friction, pile stiffness, wear resistance and recovery capacity.

8. Method as claimed in claim 7, characterized in that at least one film is used with moisture absorbing properties.

9. Method as claimed in claim 8, characterized in that use is made of a "super absorber", for example a cross linkable sodium polyacrylate.

10. Method as claimed in claim 7, characterized in that three films are co-extruded, the middle one of which consists of a polypropylene while the outer films consist of a softer, more flexible and/or smoother material.

11. Method as claimed in claim 10, characterized in that the outer films contain linear low density polyethylene.

12. Method as claimed in claim 10, characterized in that the outer films contain polyethylene terephthalate.

13. Method as claimed in claim 10, characterized in that the outer films each have a relative thickness in the order of magnitude of 20% of the total thread thickness.

14. Method as claimed in claim 1, characterized in that use is made of frizzed threads.

15. Method as claimed in claim 14, characterized in that the frizzing of the threads is fixed by a heat treatment.

16. Method as claimed in claim 15, characterized in that the pre-frizzed threads are exposed to at least one heating up to approximately 130°C for a time period in the order of 10 minutes.

17. Method as claimed in claim 16, characterized in that use is made of steam.

18. Method as claimed in any of the foregoing claims, characterized in that the threads are subjected to a fibrillation by piercing the strip-like threads with needles.

19. Method as claimed in any of the foregoing claims, characterized in that the threads or the completed artificial grass are subjected to an after-treatment for applying to said threads a coating layer containing a smoothing substance, which contains polytetrafluoroethylene or a material on a silicon base.

20. Method as claimed in claim 19, characterized in that a watery dispersion is made of the smoothening substance, which is applied to the threads by spraying or other suitable process, and the water is allowed to evaporate.

21. Artificial grass obtained by application of a method as claimed in any of the foregoing claims.

## Revendications

1. Procédé de fabrication d'une herbe artificielle, se composant d'une sous-couche et de fils de poils, de type en bande, encastrés dans ladite sous-couche, lesquels fils, comme de l'herbe, dépassent de la sous-couche sur un côté de cette dernière, dans lequel l'on utilise un polymère comme matière première pour les fils, caractérisé en ce que l'on ajoute à ladite matière première un deuxième matériau présentant une composition différente et réduisant le coefficient de friction.

2. Procédé selon la revendication 1, caractérisé en ce que la matière première est un polypropylène.

3. Procédé selon la revendication 1, caractérisé en ce que l'on mélange du polytétrafluoréthylène ou du polyéthylènetéréphtalate avec le polymère, par exemple sous forme d'un mélange maître.

4. Procédé selon la revendication 3, caractérisé en ce que le mélange est effectué dans une proportion de l'ordre de 50%/50% .

5. Procédé selon la revendication 3, caractérisé en ce que la quantité de polytétrafluoréthylène est choisie de telle sorte que la quantité ainsi obtenue représente approximativement 2-7% du poids total des fils.

6. Procédé selon la revendication 1, caractérisé en ce que , pour la fabrication des fils, les deux matériaux sont extrudés en même temps.

7. Procédé selon l'une quelconque des revendications précédentes, caractérisé en ce que les fils sont fabriqués par co-extrusion d'un certain nombre de feuilles afin d'obtenir les propriétés mécaniques requises, tel que le coefficient de friction, la rigidité des poils, la résistance à l'usure et le pouvoir de récupération.

8. Procédé selon la revendication 7, caractérisé en ce que l'on utilise au moins un film présentant des propriétés d'absorption de l'humidité.

9. Procédé selon la revendication 8, caractérisé en ce que l'on utilise un "super absorbant", par exemple, un polyacrylate de sodium réticulable.

10. Procédé selon la revendication 7, caractérisé en ce que trois feuilles sont coextrudées, la feuille du milieu se composant de polypropylène tandis que les feuilles externes se composent d'un matériau plus doux, plus souple et/ou plus lisse.

11. Procédé selon la revendication 10, caractérisé en ce que les feuilles externes contiennent du polyéthylène linéaire à faible densité.

12. Procédé selon la revendication 10, caractérisé en ce que les feuilles externes contiennent du polyéthylènetéréphtalate.

13. Procédé selon la revendication 10, caractérisé en ce que les feuilles externes présentent chacune une épaisseur relative de l'ordre de 20% de l'épaisseur totale des fils.

14. Procédé selon la revendication 1, caractérisé en ce que l'on utilise des fils bouclés.

15. Procédé selon la revendication 14, caractérisé en ce que le bouclage des fils est fixé par un traitement thermique.

16. Procédé selon la revendication 15, caractérisé en ce que les fils pré-bouclés subissent un chauffage d'une température pouvant atteindre 130°C pendant une durée de l'ordre de 10 minutes.

17. Procédé selon la revendication 16, caractérisé en ce que l'on utilise de la vapeur.

18. Procédé selon l'une quelconque des revendications précédentes, caractérisé en ce que les fils subissent une fibrillation par perçage des fils de type en bande à l'aide d'aiguilles.

19. Procédé selon l'une quelconque des revendications précédentes, caractérisé en ce que les fils ou l'herbe artificielle terminée sont soumis à un traitement ultérieur consistant à appliquer auxdits fils une couche de revêtement contenant une substance d'assouplissage, qui contient du polytétrafluoréthylène ou un matériau sur une base de silicone.

20. Procédé selon la revendication 19, caractérisé en ce que l'on prépare une dispersion aqueuse de la substance d'assouplissage pour l'appliquer aux fils par pulvérisation ou selon tout autre procédé approprié, en laissant ensuite l'eau s'évaporer.

21. Herbe artificielle obtenue par l'application d'un procédé selon l'une quelconque des revendications précédentes.

## Patentansprüche

1. Verfahren zur Herstellung von Kunstgras, das eine Unterschicht und darin eingebettete, streifenähnliche Florfasern aufweist, wobei die Fasern als Gras aus einer Seite der Unterschicht vorstehen und wobei als Rohmaterial für die Fasern ein Polymer verwendet wird, dadurch gekennzeichnet, daß dem Rohmaterial ein zweites Material mit unterschiedlicher Zusammensetzung zugesetzt wird, das den Reibungskoeffizienten vermindert.

2. Verfahren nach Anspruch 1, dadurch **gekennzeichnet,** daß das Rohmaterial ein Polypropylen ist.

3. Verfahren nach Anspruch 1, dadurch **gekennzeichnet,** daß Polytetrafluoräthylen oder Polyäthylenterephthalat mit dem Polymer gemischt ist, beispielweise in Form einer Vormischung.

4. Verfahren nach Anspruch 3, dadurch **gekennzeichnet,** daß das Mischungsverhältnis in der Größenordnung von 50 % : 50 % gewählt ist.

5. Verfahren nach Anspruch 3, dadurch **gekennzeichnet,** daß die Menge von Polytetrafluoräthylen so ausgewählt ist, daß seine resultierende Menge etwa 2-7 % des Gesamtfasergewichtes trägt.

6. Verfahren nach Anspruch 1, dadurch **gekennzeichnet,** daß zur Herstellung der Fasern beide Materialien gleichzeitig extrudiert werden.

7. Verfahren nach einem der vorstehenden Ansprüche, dadurch **gekennzeichnet,** daß die Fasern durch Co-Extrusion einer Anzahl von Filmen hergestellt werden, um die erforderlichen mechanischen Eigenschaften wie Reibungskoeffizient, Florsteifigkeit, Verschleißfestigkeit und Erholungsvermögen zu erhalten.

8. Verfahren nach Anspruch 7, dadurch **gekennzeichnet,** daß zumindest ein Film mit feuchtigkeitsabsorbierenden Eigenschaften verwendet wird.

9. Verfahren nach Anspruch 8, dadurch **gekennzeichnet,** daß ein "Superabsorber" verwendet wird, beispielsweise ein kreuzverbindbares Natriumpolyacrylat.

10. Verfahren nach Anspruch 7, dadurch **gekennzeichnet,** daß drei Filme co-extrudiert werden, von denen der mittlere aus Polypropylen besteht, während die anderen Filme aus einem weicheren, flexibleren und/oder glatteren Material bestehen.

11. Verfahren nach Anspruch 10, dadurch **gekennzeichnet,** daß die äußeren Filme lineares Polyäthylen mit niedriger Dichte enthalten.

12. Verfahren nach Anspruch 10, dadurch **gekennzeichnet,** daß die äußeren Filme Polyäthylenterephthalat enthalten.

13. Verfahren nach Anspruch 10, dadurch **gekennzeichnet,** daß die äußeren Filme eine relative Dicke in der Größenordnung von 20 % der Gesamtfaserdicke aufweisen.

14. Verfahren nach Anspruch 1, dadurch **gekennzeichnet,** daß gekräuselte Fasern verwendet werden.

15. Verfahren nach Anspruch 14, dadurch **gekennzeichnet,** daß die Kräuselung der Fasern durch eine Wärmebehandlung fixiert wird.

16. Verfahren nach Anspruch 15, dadurch **gekennzeichnet,** daß die vorgekräuselten Fasern zumindest einer Aufwärmung auf etwa 130 °C für eine Zeitspanne in der Größenordnung von 10 Minuten ausgesetzt werden.

17. Verfahren nach Anspruch 16, dadurch **gekennzeichnet,** daß Dampf verwendet wird.

18. Verfahren nach einem der vorstehenden Ansprüche, dadurch **gekennzeichnet,** daß die Fasern einer Faserbildung durch Durchstechen der streifenähnlichen Fasern mit Nadeln ausgesetzt werden.

19. Verfahren nach einem der vorstehenden Ansprüche, dadurch **gekennzeichnet,** daß die Fasern oder das fertiggestellte Kunstgras einer Nachbehandlung ausgesetzt werden zum Anbringen einer Deckschicht an die Fasern, die eine Gleitsubstanz enthält, die Polytetrafluoräthylen oder ein Material auf Siliconbasis enthält.

20. Verfahren nach Anspruch 19, dadurch **gekennzeichnet,** daß eine wässrige Lösung aus der Gleitsubstanz hergestellt wird, die den Fasern durch Sprühen oder andere geeignete Prozesse zugeführt wird, und daß man das Wasser verdampfen läßt.

21. Kunstgras, das mit einem Verfahren nach einem der vorstehenden Ansprüche hergestellt wurde.
